

# UNITED STATES PATENT OFFICE.

JOHN W. SPENCER, OF NEWBURN, ENGLAND.

## MANUFACTURE OF STEEL.

No. 863,763.

Specification of Letters Patent.

Patented Aug. 20, 1907.

Original application filed July 31, 1903, Serial No. 167,782. Divided and this application filed October 29, 1904.  
Serial No. 230,578.

*To all whom it may concern:*

Be it known that I, JOHN W. SPENCER, a subject of the King of Great Britain, residing at Newburn, England, have invented certain new and useful Improvements in the Manufacture of Steel, of which the following is a specification.

The object of this invention is the manufacture of improved steel wherein valuable properties are obtained rendering such steel of greater utility for boiler plates, 10 ship plates, and all classes of forgings such as are made from so-called mild and medium hard steel.

This application is a division of the U. S. application Serial No. 167,782, filed July 31, 1903, covering my method of manufacturing steel.

15 According to my invention I add to all kinds of mild and medium hard steels containing carbon from .05% up to .25%, a larger proportion of silicon than has hitherto been used commercially.

It is common knowledge that silicon has been and 20 is used for such purposes as conferring solidity upon steel castings and ingots, and in much larger proportions for the manufacture of the harder classes of steel, such as spring steel and tool steel.

It is the special object of my invention to utilize the 25 valuable properties conferred upon mild and medium hard steels by the addition of proportions of silicon varying from .75% up to 2%. By this means the tensile strength and elastic limit of the resulting steel are enormously increased without impairing its ductility 30 thus rendering it of much greater value for many purposes.

Not only does the steel made according to my invention possess improved strength and ductility but it also possesses other marked physical properties of advantage which are shown by the bending and fatigue tests.

For ship plates the strength is so much increased that the thickness of the plates may be so much reduced as to make a great difference in the cost of construction and carrying power of the vessels. For boiler 40 plates and forgings the strength is so much increased that an increased factor of safety may be obtained where it may not be considered expedient to reduce the weight.

My present invention consists, therefore, in utilizing 45 this valuable property of silicon and applying it to ob-

tain such results as are only at present attainable commercially by the use of nickel which is much more expensive to add than silicon and which is attended by certain disadvantages not possessed by the silicon.

One of the great advantages in the use of silicon in 50 such proportions as are hereinbefore specified, for increasing the strength without loss of ductility, is, that plates and forgings may be obtained—practically free from surface defects, a well known difficulty in the use of nickel for such a purpose. The steel which has been 55 improved by the addition of silicon is also easily welded, which renders it particularly suitable for plates.

Hitherto the special addition of such large proportions of silicon as are described in my invention has been of scientific interest only and to the best of my 60 knowledge no one has yet attempted to apply it commercially to improve the milder qualities of steel at present in use, and it is this which I particularly claim to have discovered.

In carrying out my invention I proceed to melt a 65 charge of suitable materials such as scrap and pig iron either alone or as a mixture in a crucible, open hearth, or other furnace, or Bessemer or other converter. After the charge of pig-iron and scrap has been melted and worked down or purified, as is usual in the Siemens or 70 Bessemer processes, I then introduce the desired proportion of silicon, or silicon alloy either into the furnace, or into the ladle, after which the mixture is cast into ingots or other desired form.

In making my improved steel in this manner manganese may be added in the usual way or in certain cases it may be dispensed with.

Having now particularly described and ascertained the nature of my said invention, and in what manner the same is to be performed, I declare that what I 80 claim is:

As a new article of manufacture, a steel consisting of iron, .05 to .25 percent of carbon and .75 to 2 percent of silicon.

In testimony whereof I have hereunto set my hand in 85 presence of two subscribing witnesses.

JOHN W. SPENCER.

Witnesses:

W. H. NIXON,  
D. OTTO LILLY.